

Patented Nov. 15, 1927.

1,648,954

# UNITED STATES PATENT OFFICE.

JOHN WESLEY MARDEN, OF EAST ORANGE, NEW JERSEY, ASSIGNOR TO WESTINGHOUSE LAMP COMPANY, A CORPORATION OF PENNSYLVANIA.

## PRODUCTION OF RARE METALS AND ALLOYS THEREOF.

No Drawing.

Application filed September 29, 1921. Serial No. 504,154.

This invention relates to the preparation of metals, more especially of the rare metals. My invention is more particularly adapted for the production of metals such as zirconium, uranium, thorium, titanium, tantalum, molybdenum, chromium, vanadium, tungsten, etc., often known as the refractory metals, beryllium, the rare earth metals, and the like.

10 Metals of the character mentioned above, particularly the refractory metals, are obtainable with great difficulty, especially on a commercial scale, in their pure or elemental state. This, to a great extent, is probably 15 due to such metals, as well as their compounds, having high melting points and to the considerable difficulty encountered in separating such metals from the substances with which they may be compounded.

20 Furthermore, even when such metals have been obtained in the elemental form, they are maintained in such form with great difficulty because they readily oxidize in pure water or in the air. For instance, uranium 25 slowly interacts with water to form an hydroxide or oxide, and, because of the ready solubility of that metal in dilute acids, it is very difficult to segregate the oxide or hydroxide thus formed. As another example 30 of such activity, zirconium may be cited, even though that metal in the powder state is quite insoluble in hydrochloric, nitric or sulphuric acids. Zirconium powder forms the hydroxide after standing in water some

35 time. What is true of the metals mentioned above is undoubtedly true of thorium, for, although the oxide of that metal may be reduced by means of calcium or other means, it is difficult to treat the metal powder with 40 water and dilute acid for the removal of impurities and still have an oxide-free metal. As a matter of fact, thorium tarnishes in moist air. If thorium powder is sealed up in air containing but a little moisture, which 45 is ordinarily in the air, the oxide forms, and probably the nitride also, as a large amount of ammonia gas is formed under these conditions.

50 It will thus be seen that, where it is necessary to resort to washing or treatment with acids to obtain a pure-metal powder, small amounts of impurities are introduced. It is well known that, with such impurities present in the metal powder, it is difficult to work 55 such metals or to reduce them to a coherent

condition so that they may be readily wrought, as, for instance, for the production of metallic articles, as filaments, lead-in wires, electrodes, and the like.

60 One of the methods which has been invented by me for the production of these rare metals directly from their salts without necessitating the washing of the metal powder by water, dilute acids or exposure to the air during any step of the process, is set 65 forth in detail in my copending application, Serial Number 432,324, filed December 21, 1920, for the Preparation of rare metals. Briefly stated, this process consists in mixing the double halide salts with aluminum 70 in a metal crucible and heating the mixture in a high-frequency induction furnace under a high vacuum until the reduction is completed, the excess of salts volatilized, and the metal completely sintered to a coherent 75 mass.

When these metals are in the coherent form, they do not oxidize so readily as when in the powdered state. However, from a commercial viewpoint it may be desirable to 80 have these metals combined in such form that the purchaser need not resort to any difficult, tedious or expensive treatment steps in order to obtain the pure elemental metal therefrom. At the same time, it may 85 be desirable to have the metal in such condition that it may be worked.

It is, therefore, one of the objects of my invention to prepare compounds or alloys 90 of the metals of the character mentioned in such form that they may be readily handled in commerce without danger of oxidation or otherwise becoming contaminated, and which, at the will of the purchaser, may be reduced to their pure elemental form without difficulty and without danger of contamination and also in such condition that they may be worked, if desired.

In practicing my invention, I prepare a compound of the rare metal with another 100 substance from which the rare metal may be readily reclaimed, the compound being stable under normal conditions so that the likelihood of the rare metal becoming contaminated through oxidation or otherwise, is reduced to a minimum. More particularly, the method comprises forming an alloy of 105 the rare metal and aluminum, which alloy is, in most cases, more stable than the metal itself, and, when it is desired to obtain the 110

rare metals, of heat-treating the alloy or compound to distill away the aluminum in the absence of air or any other contaminating agency or substance.

- 5 The first step in my method comprises obtaining the compound or alloy. I have successfully used two different methods for accomplishing this purpose, one being an alumino-thermic process based upon the 10 Goldschmidt principle which, with certain rare metals and under varying conditions, is found to be preferable, while the other relates to the treatment of the double halide salts of the rare metals with aluminum.
- 15 A specific example of the operation of my invention for the production of rare-metal alloys in which recourse is had to the alumino-thermic mode of treatment, may be as follows: I prepare a charge composed of 20 a mixture of uranium oxide, potassium chlorate and aluminum powder. The proportions are so arranged that the potassium chlorate adds heat to the reaction and a one-hundred-percent excess of aluminum is used 25 in order to form the alloy. If only a small quantity of the aluminum is used, the reduction of the rare metal only will be effected and the alloy will not be formed. The ingredients are carefully mixed on a paper 30 with a spatula and slowly poured into a graphite or fire-clay crucible of proper size. Considerable care should be exercised in preparing the mixture, otherwise an explosion may occur. The crucible into which 35 the mixture is poured should be cold, otherwise there is danger to the operator. A primer, comprising a mixture of finely powdered magnesium or aluminum and potassium chlorate, is placed on top of the mixture 40 in the crucible and this material is ignited by means of a fuse made of magnesium ribbon in the customary manner. The purpose of adding the potassium chlorate is to furnish an oxygen-containing substance 45 which will furnish the necessary amount of heat for the reaction, therefore, any such compound may be used. Barium peroxide may be employed in place of the potassium chlorate, either in the charge or in the 50 primer or in both. Upon ignition, the charge goes off with an evolution of a sufficient amount of heat to completely melt the mixture and cause the aluminide to separate at the bottom free from the slag. If approximately equal proportions of the rare-metal oxide and potassium chlorate, with 55 about fifteen times the quantity of aluminum, is used in preparing the mixture, the required amount of heat will be evolved not 60 too rapidly. This may be controlled to a considerable extent by the fineness of the aluminum powder used. As a rule, the finer the powder the more rapid the evolution of heat. A 40-mesh aluminum powder 65 is preferable.

An important consideration in successfully utilizing the process is to retain the heat within the crucible as long as possible in order to allow the metal alloy to separate at the bottom free from the slag. Therefore, it is preferable to pack the crucible in which the reaction takes place in sand, Sil-osel, or some other heat insulator. Another consideration in carrying the reaction to a successful completion is to avoid the introduction of silicon into the metal for the reason that silicon readily alloys with aluminum, and, once it is introduced into the product, it cannot be separated. To avoid this contamination and to obtain a pure alloy of uranium and aluminum, it is preferable to line the inside of the crucible with magnesia or carbon or some other refractory material, so that there will be no chance of silicon getting into the aluminum alloy. A mixture of coal tar and magnesia forms a desirable lining.

After the reaction is complete and the mass has cooled, it will be found that the alloy has formed into a button at the bottom of the crucible. This button is of metal and may be broken away from the crucible and the slag and subsequently crushed or comminuted into a fairly fine powder. The powder may be then purified in any desired manner to recover the uranium-aluminum alloy, or aluminide, from the other substances formed during the reaction, and the excess of aluminum. In the experiments I have conducted in obtaining this alloy, I found it preferable to purify the powder by treating with a fairly strong solution of caustic soda. This removes the excess of aluminum not alloyed with the uranium or other metals. I then decant the caustic-soda liquor away and wash the residue of crystalline aluminide with water and treat with dilute hydrochloric acid to remove all of the hydroxide and acid-soluble materials from the alloy. The fine crystalline alloy is filtered and dried in the customary manner. The aluminide thus obtained may be sold in commerce or else screened to remove coarser particles if a finer grade is desired.

The alloy of uranium and aluminum obtained by following the foregoing process is a white finely divided coherent metal, free from any oxide or carbon, and is composed of small platelets, probably belonging to the monoclinic system of crystallization. It is more stable toward dilute hydrochloric acid than either of its constituent metals. The uranium, combined with the aluminum in the form of an alloy, will be preserved from tarnishing or becoming contaminated, and, when it is desired to obtain or reclaim it, the process hereinafter described may be practiced.

The other method which I have used and found especially desirable in producing the

rare-metal alloys will now be described, with thorium as the specific example; a halide salt of thorium, as thorium ammonium chloride, is prepared preferably by the process invented by me and fully described in an application for patent, Serial #498,397, filed September 3, 1921, for the Preparation of metals and their halides. Briefly stated, that process involves the treatment of the hydrated salts of the rare metals with a displacing substance, as ammonium chloride, which, when added to a solution in which the hydrated salt has been dissolved, will displace the water in the positive radical. The solution is then evaporated to dryness to liberate the water and part of the ammonium chloride. The residue is thorium ammonium chloride, which is the substance I employ in preparing the alloy according to this method.

In order that the halide salt may be obtained perfectly dry, it should be heated to a temperature of about 100° C. before proceeding with my process. The dried salt is placed in a graphite crucible and covered with a previously fused and cooled mixture of sodium and potassium chlorides or fluorides or other halogen-containing alkali compounds. The crucible, with the mixture therein, is placed within a furnace and the temperature is raised until the mixture is fused to a clear liquid. In order to prevent the thorium or aluminum from becoming oxidized or otherwise contaminated, a slow current of carbon tetrachloride vapor, or other chlorine-containing reducing agent, is passed into the top of the crucible. When the fusion is complete, approximately several times the weight of aluminum necessary to make the reduction, which will be termed hereinafter as an excess of aluminum, is added to the fused mixture in successive small quantities.

After the reaction is complete and the excess of aluminum has been added, the heating is continued for about twenty minutes or until the aluminum-thorium alloy mass collects and separates itself from the fused salt or slag at the bottom of the crucible in the form of a button or globule. The thorium-aluminum button is separated from the fused salt by washing away the salt with water, and, after removing the button, it may be comminuted into a fairly fine grade of powder in any convenient manner. The aluminum which is in excess and which has not alloyed with the thorium or other metals is then dissolved by treating the powder with a fairly strong solution of caustic soda. The caustic-soda liquid is decanted away and the residue of crystalline aluminide washed first with water and then treated with dilute hydrochloric acid to remove all the hydroxide and acid-soluble materials from the alloy. The thorium-aluminum alloy thus formed is

in small platelets which will be found to be more resistive to the action of dilute acids and chemical agents than thorium itself.

Should the thorium metal be desired, the process just described may be employed, the only alteration necessary being in the amount of aluminum added to the mixture, which should be about one-fourth or one-fifth of the quantity required to form the alloy. In purifying the pure metal to separate it from the fused salts after the mass has been sufficiently fused and heat treated, it need only be washed with water to dissolve the salts, treated with dilute nitric acid, filtered and dried in any customary manner.

Aluminum alloys of any of the metals hereinbefore enumerated are considerably more stable in the air or moisture than any of the constituent metals, and, in view of that fact alone, the preparation of the rare metal in such form furnishes an ideal way to preserve the metal from tarnishing or becoming contaminated. It is preferable, however, in thus preserving these metals, that the metals or substances with which they may be compounded or alloyed have such properties that the rare metal may be readily separated or reclaimed without involving any expensive, tedious or involved chemical-treatment steps. When the rare metal is combined with a metal having a low volatilization temperature, the former may then be obtained by merely distilling the other metal. Inasmuch as I have found this type of alloy preferable for the purpose in hand, the following specific example will be confined thereto in explaining the process for reclaiming the rare metal.

The finely divided crystalline alloy is first screened to remove any coarse particles which were not disintegrated by the caustic soda or dilute acid. The fine alloy powder is compressed into a disk or rod in order that the material may be more readily handled for subsequent treatment in the furnace, and, in this form, is placed in a furnace, preferably of the type described in the copending application of Rentschler, Serial #430,118, filed December 13, 1920, on Furnaces, and assigned to the Westinghouse Lamp Company. The rod is slowly brought to the temperature at which the aluminum will distill off, and such treatment continued until all the aluminum is liberated.

If the material is heated in a crucible, it may be heated up rapidly and the aluminum boiled away, but, if it is heated in the form of a disk in a high-frequency furnace, such as is described in the application heretofore referred to, or in the form of a rod by passing the current directly through it, as by the type of furnace described in the copending application filed by Rentschler and Mar-don, Serial #488,230, filed July 28, 1921, and assigned to the Westinghouse Lamp

Company, the heating must be done very slowly indeed, in order to boil the aluminum away without melting the alloy or without shrinking so rapidly as to crack the material.

The slow heat treatment has an additional beneficial effect on the rare metal in that it causes the particles of which it is composed to adjust themselves in certain definite relationship to render the material ductile and properly condition it for mechanical treatment, as swaging, rolling, and the like. That is, the metal may be wrought or satisfactorily worked into any desired form.

15 In order that the metal shall not become contaminated during the heat treatment, it is preferable to perform this operation in a vacuum or inert environment. The higher the vacuum used the purer the metal will be, and, therefore, in my work I used the highest attainable vacuum as obtained by means of a diffusion pump.

Although I have specifically described certain modes of treatment and selected certain metals in describing such processes, I desire it to be understood that I do not wish to be confined thereto but reserve the right to consider any other processes or materials which come within the scope of the appended claims as falling within the spirit of my invention.

What is claimed is:

1. A method of preparing metal alloys which comprises fusing a salt of a metal with a mixture of several of the alkali-metal halides, adding a large excess of a reducing metal slowly to the fused mixture and, after the reaction is complete, heating until the alloy separates from the fused salt and treating out the salt and the excess aluminum.

2. A method of preparing metal alloys which comprises fusing a salt of a metal with a mixture of sodium and potassium halides, adding a large excess of aluminum to the fused mixture and, after the reaction is complete, heating until the alloy separates from the fused salt and treating out the salt and the excess aluminum.

50 3. A method of preparing rare-metal alloys which comprises fusing a mixture of a salt of a rare metal and a mixture of sodium and potassium chlorides, adding aluminum to the mixture until there is a large excess, continuing the heat treatment until the alloy separates from the fused salt and treating out the salt and the excess of aluminum.

60 4. A method of preparing alloys of thorium which comprises fusing a double halide of thorium and a mixture of sodium and potassium chlorides, adding a reducing agent to the fused mass, a little at a time, until there is a considerable excess, continuing the heat treatment until the alloy of

thorium and aluminum separates from the fused salts and treating out the fused salts and excess of aluminum.

5. A method of preparing metals which comprises mixing a salt of a metal with more than the theoretical amount of a metal necessary to completely reduce said salt, heating the same to reaction temperature, and treating out the substances thus formed except the alloy and heating the alloy in an inert environment at a sufficiently high temperature to volatilize the second metal.

6. A method of preparing metals which comprises mixing a salt of a rare metal with more than the theoretical amount of a metal so necessary to completely reduce said salt, heating the same to reaction temperature, treating out the substances thus formed, except the alloy, and heating the alloy thus formed in an inert environment at a sufficiently high temperature to volatilize the second metal.

7. A method of preparing metals which comprises fusing a salt of a metal with a mixture of several of the alkali-metal halides, adding a large excess of a reducing metal slowly to the fused mixture, and, after the reaction is complete, heating until the alloy separates from the fused salt, treating out the salt and the excess aluminum and heating the alloy in an inert environment at a sufficiently high temperature to volatilize the second metal.

8. A method of preparing metals which comprises fusing a mixture of a salt of a rare metal and sodium and potassium halides, adding a large excess of aluminum to the fused mass, continuing the heat treatment until the alloy separates from the salt and treating out the salt and any excess aluminum and heating the alloy in an inert environment at a sufficiently high temperature to volatilize the second metal.

9. A method of preparing metals which comprises forming an alloy of a metal with another metal, such as aluminum, by fusing a salt of the first metal with a mixture of a plurality of alkali halides, adding a large excess of a reducing metal slowly to the fused mass, continuing the heat treatment after the reaction is completed until the alloy separates from the fused salt, treating the mass to obtain the alloy and decomposing the alloy to obtain the metals by distilling away the reducing metal by heat treatment in an inert environment.

10. A method of preparing rare metals which comprises first forming an alloy of a rare metal with another metal by fusing a salt of the rare metal with a mixture of a plurality of alkali halides, such as potassium and sodium chlorides, slowly adding the second metal to the fused mixture until an excess of the metal is obtained, continuing the heat treatment until the alloy sepa-

rates from the fused salt, treating out all substances in the mass but the alloy, and, secondly, decomposing the alloy to obtain the rare metal by heat treatment in an inert environment to distill away the other metal.

11. A method of preparing thorium which comprises forming an alloy of thorium and aluminum by fusing a double halide of thorium and a mixture of sodium and potassium chlorides, adding aluminum slowly to the fused mass until there is a considerable excess, continuing the heat treatment until the alloy of thorium and aluminum separates from the fused salts, treating out the substances, other than the alloy, and heat treating the alloy in an inert environment to distil off the aluminum.

12. A method of preparing rare refractory metals which comprises forming an alloy of a rare refractory metal and a readily distillable substance and heat treating the alloy in an inert environment in such manner as to

slowly distill all the said substance away from the rare refractory metal and to cause the latter to become ductile. 25

13. A method of making refractory metals ductile which comprises forming an alloy of a refractory metal with aluminum and heat treating the alloy in an inert environment to slowly distill all the aluminum off 30 and to cause the refractory metal to become conditioned so that it may be wrought.

14. A method of making refractory metals ductile which comprises heat treating an aluminum alloy of a refractory metal in an 35 inert environment in such manner as to slowly distill all the aluminum away from the refractory metal and to cause the latter to become ductile.

In testimony whereof, I have hereunto sub- 40 scribed my name this 28th day of September, 1921.

JOHN WESLEY MARDEN.